

April 22, 1952

M. T. ORINIK

2,593,912

PHOTOGRAPHIC FILM CONTAINING HARDENED GELATIN

Filed Nov. 19, 1948



FIG. 1



FIG. 2

INVENTOR  
MICHAEL T. ORINIK

By *Henry W. Connelly*  
*Henry B. Elling*  
ATTORNEYS

## UNITED STATES PATENT OFFICE

2,593,912

PHOTOGRAPHIC FILM CONTAINING  
HARDENED GELATINMichael T. Ornik, Binghamton, N. Y., assignor  
to General Aniline & Film Corporation, New  
York, N. Y., a corporation of Delaware

Application November 19, 1948, Serial No. 61,137

5 Claims. (Cl. 95—9)

1

This invention relates to photographic film and particularly to an improved photographic film containing hardened gelatin.

It is known that photographic film is prepared by the coating of a gelatino silver halide emulsion layer on a transparent film base. Cellulose nitrate has been used primarily because of its highly desirable physical properties, such as strength, rigidity, and toughness. It possesses, however, one outstanding disadvantage in that it is extremely inflammable. With the advent of amateur processing and projection of 8 mm. and 16 mm. film, it has been desirable to provide a non-inflammable film, and the photographic industry to achieve this end has been using cellulose ester film bases. The normal cellulose acetate of commerce, containing 56-58% of combined acetic acid content, has been found inferior photographically to cellulose nitrate. Cellulose esters of higher acid content have been found to be extremely difficult to process despite their more desirable photographic properties.

The principal drawback of the higher cellulose acetate acid esters (58-61% of combined acetic acid) has been the difficulty in applying the gelatino silver halide emulsion layer and associated non-curl, filter, and anti-halation layers to insure adhesion between the coated layers and the film base proper. Slight variations in temperature, humidity, hardness, etc., give rise to reticulation, peeling, and frilling of the coated layers from the film base.

It is the practice in the photographic art to apply a special layer, known as the subbing layer, to promote adhesion of the gelatino silver halide emulsion layer and other auxiliary layers. Materials suggested for the subbing of a photographic film base include cellulose nitrate-plasticizer mixtures, gelatin-cellulose nitrate mixtures, modified gelatin layers over-coated with plain gelatin, etc.

From a subbing standpoint, many attempts have been made to harden the gelatin in a subbing solution chemically to reduce its moisture susceptibility and improve other physical characteristics. The commonly employed hardening agents, such as formaldehyde, glyoxal and the like, give sometimes the impression of showing poor solubility in the usual subbing composition by causing an electrolytic precipitation of the gelatin from the subbing solution. Another difficulty encountered is that the gelatin subbing compositions are strongly acid in nature and many of the organic hardening agents employed operate best in neutral or alkaline subbing solu-

2

tions or dispersions. For these reasons, the art has always been of the belief that all organic hardening agents are inoperative in the usual gelatin subbing compositions. This belief was based on the assumption that the hardening action of the organic hardening agents is strongly inhibited by the presence of either acid or organic solvent in the subbing solution or dispersion.

10 Inorganic salts of trivalent chromium, such as chromium chloride, chromium nitrate, chrome alum and the like, have also been suggested as hardening agents in gelatin subbing compositions. Their presence in gelatin subbing solutions or compositions also causes electrolytic precipitation of the gelatin over a period of time so that the resulting subbing solution loses strength on standing and subtracts from the adhesive properties between the film base and the adjacent gelatin emulsion or non-curl layers. Although it is possible to secure sufficient adhesion of the coated photo-sensitive layers for short periods of time, it has been found that storage for periods of time greater than six months is deleterious to the product as a whole.

The present invention has as an object to overcome the above-mentioned difficulties and to provide an improved photographic film containing hardened gelatin.

30 Another object is to provide a non-desensitizing, non-corrosive subbing solution of hardened gelatin for subbing cellulose derivative film supports.

35 A further object is to provide a gelatin subbing composition free from electrolytic precipitation.

Other objects and advantages will appear from the following description.

I have found that of all the organic hardening agents employed for hardening gelatin-subs and gelatino silver halide emulsion layers, formaldehyde and glyoxal in specific amounts function most satisfactorily as hardening agents for gelatin subbing solutions. These hardening agents when employed in specific amounts or concentrations possess none of the disadvantages referred to above. The formaldehyde or glyoxal hardening agents are incorporated into the gelatin subbing composition containing gelatin, water, dispersing medium such as an organic acid, acetic acid and the like, cellulose derivative, as will be pointed out hereinafter, and an organic solvent or a mixture of such solvents.

The gelatin subbing compositions are prepared by adding the formaldehyde or glyoxal to

a gelatin dispersion containing gelatin, water and a dispersing medium and thereafter adding the dispersion to an organic solvent, such as, for example, methanol, ethanol, acetone, methyl acetate, methyl cellosolve, or a mixture of such solvents, or by adding the formaldehyde or glyoxal to the finished gelatin subbing composition, i. e., containing the organic solvents or mixtures thereof. The solution thus obtained is deposited on one or both sides of a cellulose derivative film base in any convenient manner, the subbing operation preferably being carried out in connection with or as a part of the process of making the film support itself. The gelatin subbing solutions made up as above described are clear dispersions from which the gelatin is not precipitated by either the formaldehyde or glyoxal.

The amount or concentration of formaldehyde or glyoxal to be added to the gelatin subbing solution depends on the amount of the organic hardening agent used in any one of the adjacent gelatin layers such as in the gelatino silver halide emulsion layer, the non-curling or anti-halation layer. The organic hardening agent employed in any one of the adjacent layers may be any one of the reactive aldehyde or keto compounds commonly employed for this purpose, such as, for example, formaldehyde, glyoxal, acetaldehyde, hydroxyldehydes, such as glycolaldehyde, keto-aldehydes, such as methylglyoxal, diacetyl, and the like. Of these, glyoxal and formaldehyde are preferred. Optimum adhesion is obtained when the amount of formaldehyde or glyoxal in the gelatin subbing solution is equal to or is in limited excess of that employed in any one of the adjacent layers. By careful control of the amount of formaldehyde or glyoxal in the gelatin subbing layer, I have found that there exists a critical relationship between the amount of organic hardener in the gelatino silver halide emulsion layer and the amount of glyoxal or formaldehyde in the gelatin subbing layer. When the amount of hardener in the gelatin subbing layer deviates from the critical optimum range, deleterious effects, such as poor adhesion, frilling, and artificial aging with consequent photographic deterioration of the emulsion results. The critical relationship which I have discovered is that the proportion of formaldehyde or glyoxal, in relation to the amount of dry gelatin, in the gelatin subbing solution or composition must be at least equal to and should not exceed by more than 5 parts per thousand the proportion of organic hardening agent, in relation to the amount of dry gelatin, in the adjacent gelatin layer. For example, if the amount of the organic hardening agent in the adjacent gelatin layer is 0.4% (based on the weight of dry gelatin), the amount of formaldehyde or glyoxal in the gelatin subbing layer should be from 0.4 to 0.9% (based on the weight of dry gelatin in the subbing composition). This relationship with respect to amounts or concentrations is so critical that any deviation will subtract from the adhesive properties of the subbing composition and will give rise to the condition known as frilling.

The amount of organic hardening agent which may be added to gelatinous silver halide layers normally varies from 0.5 gram to 100 grams per kilogram of dry gelatin, and depends on the type of hardener and the strength of the gelatin solution used.

When formaldehyde or glyoxal are employed as hardening agents for gelatinous silver halide emulsions or non-curling layers, amounts rang-

ing from 0.5 gram to 7.5 grams of hardener per kilogram of dry gelatin are commonly preferred. For all practical purposes, I have found that when the ratio of formaldehyde or glyoxal to gelatin in the subbing layer is just equal to the ratio of organic hardener to gelatin in the adjacent emulsion or non-curling layer, all the layers possess mechanical characteristics which promote normal flexing without cracking, or distorting any one of the layers. A slight excess of formaldehyde or glyoxal in the gelatin subbing layer within the foregoing limits seems to cause a more positive bonding action at the interface.

The cellulose derivative used in the gelatin subbing composition in accordance with this invention and to which said compositions are applied are cellulose nitrate, cellulose acetate, cellulose triacetate, cellulose formate, cellulose propionate, cellulose butyrate, cellulose acetate-butyrate, cellulose acetate-propionate, and the like, the partially hydrolyzed derivatives thereof such as hydrolyzed cellulose acetate, hydrolyzed cellulose acetate-propionate, and the like, and ethers of cellulose such as ethyl ether, benzyl ether and the like.

It will be appreciated that each different type of cellulose ester, hydrolyzed derivative ester and mixtures thereof requires slightly different solvent or solvent combination. The solvent or solvent mixture employed is such that it will have a solvent or at least a softening or swelling action on the film base so as to stick or anchor the gelatin upon the area of the cellulose derivative film support which has been softened or swollen. For example, with a cellulose acetate base, a low molecular weight alcohol, e. g., methanol, ethanol or the like, or a ketone such as acetone or a mixture of 3 parts of acetone to 1 part of alcohol may be employed. With cellulose acetate-propionate film base, an alkyl ester such as, for example, methyl acetate, ethyl acetate, butyl acetate, and the like, either alone or with methanol or 1,4-dioxane may be effectively employed. Such solvents or mixtures thereof employed for the ether cellulose derivative film supports are well known to those skilled in the art and a further disclosure of them need not be made herein. It may be mentioned at this point that the nature of the gelatin dispersing medium solvent or solvent mixture is immaterial to the practice of the present invention so long as the dilute dispersing medium, whether it be an organic acid, heterocyclic nitrogenous base, lactone, or the like, disperses the gelatin in water, and the solvent or solvent mixture wets or bites into the cellulose derivative. Since materials suitable for the film base and their solvent proportions are well known no difficulty is presented in selecting a suitable solvent or solvent mixture for use in the gelatin subbing compositions.

The gelatin subbing compositions of the present invention are not only useful for the subbing of the foregoing cellulose derivative film supports, but are also useful in subbing cellulose derivative film supports containing suspended pigments of an organic or inorganic nature or both. The gelatin subbing compositions are also useful in subbing cellulose film supports for the application of non-curling and anti-halation layers.

In the accompanying drawing, the two figures are enlarged section views of a photographic film having gelatin subbing layers prepared in accordance with the present invention.

Figure 1 represents an embodiment of the invention in which the gelatin subbing layer is in-

## 5

terposed between the silver halide emulsion and support.

Figure 2 represents an embodiment of the invention in which the gelatin subbing layer is deposited on both sides of the support.

In Figures 1 and 2, 1 is the support, 2 the gelatin subbing layer containing either formaldehyde or glyoxal as the hardening agent, 3 the gelatino silver halide emulsion layer containing an organic hardening agent, 4 a gelatino silver halide emulsion layer, and 5 the non-curling or anti-halation layer containing either formaldehyde or glyoxal.

The following specific examples illustrate several of the various methods of applying the gelatin subbing compositions and it will be understood that these examples merely represent the preferred embodiments and are not to be considered as limitative. All parts and percentages are by weight.

*Example I*

A film base of cellulose acetate having a combined acetic acid content of 59% was coated with the following gelatinous substrative composition:

|                                              | Parts |
|----------------------------------------------|-------|
| Gelatin                                      | 8     |
| Water                                        | 20    |
| Acetic acid                                  | 1.2   |
| Glyoxal                                      | 0.02  |
| Cellulose acetate (56% combined acetic acid) | 6     |

The foregoing dispersion was added to a mixture consisting of 400 parts of methyl alcohol and 600 parts of acetone to make a clear subbing solution.

After the subbing layer had dried, an acid type, gelatino silver halide emulsion layer, in which the concentration of formaldehyde hardener is 2.5 parts per 1000 parts of gelatin on the dry basis, was coated directly thereon. After exposure, developing, and processing, the emulsion adhered tenaciously to the cellulose acetate film support and the processed film showed no frilling.

*Example II*

A film base of cellulose acetate-propionate having an acetyl content of 30% and a propionyl content of 13.5%, was coated on both sides with the following subbing composition:

|                              | Parts |
|------------------------------|-------|
| Gelatin                      | 8     |
| Water                        | 25    |
| Acetic acid                  | 1.2   |
| Formaldehyde                 | 0.06  |
| Cellulose acetate-propionate | 6     |

The foregoing dispersion was added to the same solvent mixture as in Example I to make a clear gelatin subbing solution.

After the subbing layers had dried, a non-curling gelatin layer was coated on one side and a gelatino silver halide emulsion layer coated on the other side of the subbed film. The concentration of glyoxal hardening agent in both coated layers is 5 parts per 1000 parts of gelatin on the dry basis. After storage for several minutes, both the non-curl layer and the gelatino silver halide emulsion layer showed strong adhesion to the cellulose acetate-propionate film base.

*Example III*

For coating a cellulose acetate-butyrat film base, having a combined acid ratio of 30% acetic

## 6

acid and 17% butyric acid with a gelatin, non-curling layer in which the concentration of formaldehyde hardener is 4 parts per 1000 parts of gelatin on the dry basis, the following subbing solution was employed:

|                           | Parts |
|---------------------------|-------|
| Gelatin                   | 10    |
| Water                     | 20    |
| Acetic acid               | 1     |
| Glyoxal                   | 0.04  |
| Cellulose acetate-butyrat | 7     |

The foregoing dispersion was added to a mixture consisting of equal parts of methanol and acetone to make a clear subbing solution.

The subbed photographic film bases produced according to the present invention, in addition to prompting better adhesion without frilling and peeling were found to be very satisfactory from the standpoint of physical requirements such as high strength, flexibility, and good water resistance.

I claim:

1. A photographic film comprising a cellulose derivative support selected from the class consisting of cellulose ethers and esters, a gelatino silver halide emulsion layer containing an organic hardening agent in an amount ranging from 0.5 gram to 7.5 grams per kilogram of dry gelatin and a gelatin subbing layer between said support and said emulsion layer, said subbing layer containing in addition to gelatin a dispersion of a cellulose derivative and a hardening agent of the class consisting of formaldehyde and glyoxal, the proportion of the latter hardening agent in relation to the weight of dry gelatin in said subbing layer being in an amount ranging from 0.5 gram to 12.5 grams per kilogram of dry gelatin and at least equal to and not exceeding by more than 5 grams per kilogram of dry gelatin the proportion of the organic hardening agent, in relation to the weight of dry gelatin, in said emulsion layer.

2. A photographic film according to claim 1 wherein the gelatin subbing layer contains glyoxal.

3. A photographic film according to claim 1 wherein the silver halide emulsion layer contains 5 grams of glyoxal per kilogram of dry gelatin.

4. A photographic film comprising a cellulose derivative support selected from the class consisting of cellulose ethers and esters, carrying on one side of said support a gelatino silver halide emulsion layer, and on the opposite side of said support a non-curling gelatin layer containing an organic hardening agent in an amount ranging from 0.5 gram to 7.5 grams per kilogram of dry gelatin, a gelatin subbing layer between said non-curling layer and said support, said subbing layer containing in addition to gelatin, a dispersion of a cellulose derivative selected from the class consisting of cellulose ethers and esters, and an organic hardening agent selected from the class consisting of formaldehyde and glyoxal in an amount ranging from 0.5 gram to 12.5 grams per kilogram of dry gelatin, the proportion of the latter hardening agent, in relation to the weight of dry gelatin in said subbing layer, being at least equal to and not exceeding by more than 5 grams per kilogram of dry gelatin the proportion of the organic hardening agent in relation to the weight of dry gelatin in said non-curling layer.

5. A photographic film according to claim 4  
wherein the non-curling layer contains 5 grams  
of glyoxal per kilogram of dry gelatin.

MICHAEL T. ORINIK.

**REFERENCES CITED**

The following references are of record in the  
file of this patent:

**UNITED STATES PATENTS**

|         |         |               |
|---------|---------|---------------|
| Number  | Name    | Date          |
| 723,054 | Smalley | Mar. 17, 1903 |

5 Number  
2,341,877

10 Number  
2,036

| Name             | Date           |
|------------------|----------------|
| Brunken          | Aug. 9, 1932   |
| Forstmann        | Sept. 15, 1936 |
| Nadeau           | Feb. 14, 1939  |
| Nadeau           | Jan. 27, 1942  |
| Middleton et al. | Feb. 15, 1944  |

**FOREIGN PATENTS**

| Country       | Date    |
|---------------|---------|
| Great Britain | of 1894 |